

May 23, 1939.

M. PIER ET AL.

2,159,511

## CARRYING OUT CATALYTIC REACTIONS

Filed Jan. 9, 1935

2 Sheets-Sheet 1



*Mathias Pier  
Walter Simon  
Paul Jacob*  
**INVENTORS**

11-212

BY *Hayff & Warland*

## THEIR ATTORNEYS

May 23, 1939.

M. PIER ET AL

2,159,511

CARRYING OUT CATALYTIC REACTIONS

Filed Jan. 9, 1935

2 Sheets-Sheet 2



Mathias Pier  
Walter Simon  
Paul Jacob  
INVENTORS

BY *Hauff & Marshall*  
THEIR ATTORNEYS

Patented May 23, 1939

2,159,511

# UNITED STATES PATENT OFFICE

2,159,511

## CARRYING OUT CATALYTIC REACTIONS

Mathias Pier, Heidelberg, and Walter Simon and Paul Jacob, Ludwigshafen-on-the-Rhine, Germany, assignors, by mesne assignments, to Standard-I. G. Company, Linden, N. J., a corporation of Delaware

Application January 9, 1935, Serial No. 1,022  
In Germany January 11, 1934

7 Claims. (Cl. 196—53)

The present invention relates to improvements in carrying out catalytic reactions, in particular the destructive hydrogenation of distillable carbonaceous materials.

It has already been proposed in our Patent No. 2,039,259 dated April 28, 1936 to carry out catalytic reactions with combustible carbonaceous materials, in particular destructive hydrogenations, in the presence of catalysts which have been prepared by decomposition of sulpho salts of heavy metals at an elevated temperature.

We have now found that it is advantageous to employ metal sulphides which have been obtained by a conversion of thio salts with compounds of metals different from those containing as metallic constituents only alkali metals and alkaline earth metals, in particular with heavy metal compounds, while dispersed in an inert ordinarily liquid medium, for example in aqueous solution or suspension or in the presence of organic solvents. By the term "inert" as applied in defining the liquid medium, it is understood that the liquid medium does not enter into any reaction with the compound or the salt dispersed in it other than possibly to effect the dissociation of any such compound or salt that does dissolve in it. However, it is to be understood that while the liquid medium in some specific cases may cause dissociation or ionization, it is not necessary in all cases that dissociation or ionization occur in order for the reactions embraced in this invention to properly take place. The said compounds, of course, may contain an alkali metal or alkaline earth metal, as for example alums or sodium zinc sulphate though heavy metal compounds containing no alkali metals or alkaline earth metals are preferable. The term thio salts is employed herein to mean the salts of oxygen acids of metallic elements the oxygen of which has been replaced by sulphur.

As thio salts are preferably employed those containing ammonium or alkali metals or alkaline earth metals as cation. Of particular advantage are the thio salts containing ammonium as cation.

The thio salts are obtained in known manner, as for example by leading hydrogen sulphide into aqueous solutions of salts capable of forming in said solutions or suspensions thio salts or by adding suitable sulphides to salts forming thio salts therewith. It is advantageous to employ the thio salts of copper, tin, vanadium, antimony, arsenic, molybdenum, tungsten, chromium, rhodium or germanium. These are brought together with other compounds of metals, in particular compounds of heavy metals of the 1st to the 8th groups of the periodic system, more especially the oxides, hydroxides or salts of these metals, as for example the halides, sulphates, nitrates, oxides, hydroxides, carbonates of copper, silver, zinc, manganese, aluminium, titanium, tin, lead,

vanadium, chromium, molybdenum, tungsten, uranium, magnesium, iron, nickel and cobalt, which may be employed in the dispersed state, for example in the form of their aqueous solutions or suspensions or dissolved or suspended in organic solvents. The metal compounds preferably contain a metal different from those contained in the thio salt employed. It is of special advantage to carry out the said conversion in the presence of organic solvents, such as acid amides, for example formamide, acid chlorides, for example acetyl chloride, amino acids, keto acids, esters, nitriles, amines, aldehydes, alcohols, ketones and nitro compounds. It is preferable to provide for the exclusion of water when employing the said solvents.

For the preparation of the catalysts, for example, the thio salts and also the metal compounds are wholly or partly dissolved at ordinary or elevated temperature in one or two of the said solvents. Both solutions or suspensions are then brought together at ordinary or elevated temperature and at atmospheric or increased pressure, if desired while stirring and/or leading in a volatile compound of bivalent sulphur, especially hydrogen sulphide or carbon disulphide. A sulphide is thus precipitated which contains two or more metals. For example by bringing together two solutions of which one contains dissolved ammonium thiotungstate in cyclohexylamine and the other dissolved cobalt chloride in acetone, a sulphide is precipitated consisting of cobalt tungsten sulphide. If by the action of hydrogen sulphide or carbon disulphide the metal compound is converted into the corresponding sulphide in such a manner that no conversion with the thio compound would take place, hydrogen sulphide or carbon disulphide are not employed. Solutions or suspensions of the reactants may also be combined in which more than one metal compound and/or thio salt are wholly or partly dissolved or suspended.

The sulphides formed may be dried and after-treated with gases such as hydrogen, volatile sulphur compounds or the like, at elevated temperature and at atmospheric or increased pressure, for example in the manner described in our before-mentioned Patent No. 2,039,259.

The precipitation of the sulphide may also be carried out in the presence of a carrier, as for example active carbon, active silica, active alumina, bentonite, Florida earth, bauxite, pumice, magnesite, magnesia and chromium oxide. The sulphides may also be applied to the carriers after precipitation. The catalysts may also be employed in admixture with other catalytic substances, as for example difficultly reducible metal oxides, such as zinc oxide, titanium oxide or alumina.

The said catalysts are very suitable for the

production of valuable hydrocarbons by the refining, aromatizing or splitting destructive hydrogenation of carbonaceous raw materials, such as coals, tars, mineral oils and their distillation and conversion products which as is known is effected at temperatures between 300° and 700° C., preferably between 380° and 550° C. and preferably at superatmospheric pressures above 20 atmospheres. The catalysts may be rigidly arranged within the reaction chamber or added to the initial materials to be treated in a finely divided state and preferably in small amounts. The catalysts are also suitable for the cracking of liquid carbonaceous materials or for the dehydrogenation of hydrocarbons or their derivatives.

Other catalytic reactions, such as the purification of gases, the preparation of methanol or hydrocarbons from carbon monoxide and hydrogen, the preparation of hydrogen sulphide from its elements, the preparation of hydrogen or of polymerization products from the waste gases from destructive hydrogenations or from cracking gases, and like reactions, may also be carried out with the aid of the said catalysts.

Our invention is further illustrated by the accompanying drawings and examples but our invention is not to be considered as restricted thereto. In the drawings:

30 Fig. 1 is a diagrammatic illustration of a suitable apparatus for preparing our catalyst; and

Fig. 2 is a diagrammatic illustration of a suitable apparatus for carrying out our process of destructive hydrogenation.

35

#### Example 1

A freshly prepared solution of 0.5 molecular proportion of titanium tetrachloride in benzine may be prepared as indicated in Figure 1 by adding the titanium tetrachloride and the benzine to a vessel 10 provided with a suitable stirrer 11. This solution is then gradually added to a solution of 1 molecular proportion of ammonium thio tungstate in cyclohexylamine. This latter may be obtained by supplying ammonium thio tungstate and cyclohexylamine to a vessel 12 equipped with stirrers 13. The solutions from the vessels 10 and 12 are passed through lines 15 and 16 controlled by valves 17 and 18 respectively to a vessel 19 equipped with a stirrer 20 and provided with a cooling jacket 21 through which cooling water may be circulated. The brown precipitate thus formed is filtered off by a suction filter 25 and is freed from adherent solvent by extraction with organic solvents of low boiling point, such for example as acetone or alcohol, which may be supplied from a tank 26 to a sprinkler 27 which is adapted to feed the solvent to the suction filter. After this treatment, the precipitate is passed through a steam drying chamber 30 and to an oven 31, having a mechanical feed 32 therein. Hydrogen and hydrogen sulphide are supplied to this oven at a temperature of from 300° C. to 400° C. The conveyor means molds the grey-black mass thus obtained or the mass may be molded by pressure in an hydraulic press or in a tablet-making machine.

This mass constitutes the catalyst which is placed in a tube 40, as shown in Figure 2, which is heated at about 410° C. in a current of hydrogen under a pressure of 200 atmospheres. The vapors of the gas oil (boiling between 200° C. and 350° C.) obtained by cracking from German crude oil are fed from a tank 41 and a pump 42 to a heat exchanger 43. Hydrogen is compressed

by a compressor 44 and is fed by a pump 45 to the heat exchanger 43 where it is mixed with the gas oil vapors. From the heat exchanger the gas oil vapors and hydrogen are passed to the preheater or furnace 46 by which they are raised to the temperature of 410° C. above mentioned and are passed through the catalyst in the tube 40. The treated vapors are withdrawn through a line 47, passed through the heat exchanger 43, then through a cooler 48 and separator 49 to 10 separate the benzine which may be removed by a line 50, the vapors being returned by a line 51 to the pump 45. The product thus obtained may consist of 70% of benzine which may be directly employed as motor fuel without further 15 refining and of 30% of illuminating oil.

#### Example 2

An aqueous solution of 1 molecular proportion of cobalt chloride is united with a 5 per cent aqueous solution of 1 molecular proportion of ammonium thiotungstate which has been freshly prepared in the cold state. The precipitated black compound is filtered off by suction, washed with water, dried in an atmosphere of nitrogen 25 and then aftertreated at from 350° to 360° C. in a current of dry hydrogen.

The catalyst, moulded by means of a press, is rigidly arranged in a high-pressure chamber, and a middle oil, prepared by the destructive 30 hydrogenation of mid-German brown coal, is led thereover in the form of vapor together with hydrogen under a pressure of 250 atmospheres at 430° C. A product is obtained which consists to the extent of 60 per cent of benzine free from 35 phenol. The remaining 40 per cent is led again over the catalyst together with fresh middle oil and thus converted into benzine.

#### Example 3

To a cold aqueous solution of one molecular proportion of ammonium thio molybdate is added a solution of two thirds of molecular proportions of ferrous sulphate. The iron-molybdenum sulphide thereby precipitated is dried while excluding air, treated with hydrogen at 300° C., pressed to pills and then rigidly arranged in a high pressure vessel. If the vapors of the middle oil fraction boiling between 200° and 375° C. of a mineral oil are passed together with hydrogen at 50 a temperature of 415° C. and under a pressure of 200 atmospheres over the thus prepared catalyst a product is obtained of which 60 per cent 55 consists of valuable benzine and of which the remainder represents an excellent illuminating oil.

#### Example 4

An alcoholic solution of anhydrous nickel chloride is added to a freshly prepared solution of ammonium thio vanadate in cyclo-hexylamine. The resulting precipitate is freed from cyclo-hexylamine and ammonium chloride formed by the conversion by extraction with alcohol and then dried while excluding air. The dried substance is subjected to an aftertreatment at 300° C. with hydrogen containing 25 per cent of hydrogen sulphide and is thereupon pressed to pieces and rigidly arranged in a high pressure 65 vessel. If the vapors of the benzine obtained by cracking a mineral oil rich in sulphur are passed together with hydrogen at 370° C. and under a pressure of 180 atmospheres over the thus prepared catalyst a product is obtained 70 75

which is free from gum forming substances and which contains only 0.005 per cent of sulphur.

*Example 5*

5 An alcoholic suspension of freshly prepared ammonium thio stannate is stirred for about 8 hours together with an alcoholic solution of anhydrous iron chloride present in the same molecular proportion as the ammonium thiostannate.

10 The resulting iron-tin sulphide is added in an amount of 0.1 per cent to a finely ground German gas flame coal which has been made up into a paste with a heavy oil from the destructive hydrogenation of the same coal; thereupon the 15 paste is heated in a coil together with hydrogen and under a pressure of 300 atmospheres to a temperature of 460° C. and subsequently passed through a high pressure reaction vessel which is maintained at the same temperature. In this 20 manner 96 per cent of the coal are converted mainly into liquid products.

What we claim is:

1. The process which comprises treating combustible carbonaceous materials heavier than gasoline under conditions to effect destructive hydrogenation at a temperature between 300° C. and 700° C., under superatmospheric pressure and in the presence of a metal sulphide catalyst which has been prepared by dispersing a thio 25 salt in an inert ordinarily liquid medium, said thio salt being of the form of a salt of an oxygen acid of a metallic element the oxygen of which has been replaced by sulphur, dispersing in an inert ordinarily liquid medium such a compound 30 of a heavy metal as is capable of entering into reaction with said thio salt with the formation 35 of a metal sulphide, and combining the dispersion of the said thio salt with the dispersion of said metal compound so that reaction therebetween takes place.

2. The process which comprises treating combustible carbonaceous materials heavier than gasoline under conditions to effect destructive hydrogenation, at a temperature between 300° C. and 700° C., under superatmospheric pressure and in the presence of a metal sulphide catalyst which has been prepared by dispersing a thio salt containing ammonium as cation in an inert ordinarily liquid medium, said thio salt being of the 40 form of a salt of an oxygen acid of a metallic element the oxygen of which has been replaced by sulphur, dispersing in an inert ordinarily liquid medium such a compound of a heavy metal substantially free from alkali metals and alkaline earth metals as is capable of entering into reaction with said thio salt with the formation of a metal sulphide, and combining the dispersion of the said thio salt with the dispersion of said metal compound so that reaction therebetween takes place.

3. The process which comprises treating combustible carbonaceous materials heavier than gasoline under conditions to effect destructive hydrogenation, at a temperature between 300° C. and 700° C., under superatmospheric pressure and in the presence of a metal sulphide catalyst which has been prepared by dispersing a thio salt containing ammonium as cation in water, said thio salt being of the form of a salt of an oxygen acid 45 of a metallic element the oxygen of which has been replaced by sulphur, dispersing in water such a compound of a heavy metal as is capable of entering into reaction with said thio salt with the formation of a metal sulphide, and combining the dispersion of the said thio salt with the dispersion of said metal compound so that reaction therebetween takes place.

4. The process which comprises treating combustible carbonaceous materials heavier than gasoline under conditions to effect destructive hydrogenation, at a temperature between 300° C. and 700° C., under superatmospheric pressure and in the presence of a metal sulphide catalyst which has been prepared by dispersing a thio 50 salt containing ammonium as cation in an organic solvent, said thio salt being of the form of a salt of an oxygen acid of a metallic element the oxygen of which has been replaced by sulphur, dispersing in an organic solvent such a compound of a heavy metal as is capable of entering into reaction with said thio salt with the formation of a metal sulphide, and combining the dispersion of the said thio salt with the dispersion of said metal compound so that reaction therebetween takes place.

5. The process which comprises treating combustible carbonaceous materials heavier than gasoline under conditions to effect destructive hydrogenation and in the presence of a metal sulphide catalyst which has been prepared by dispersing a thio salt in an inert ordinarily liquid medium, said thio salt being of the form of a salt of an oxygen acid of a metallic element the oxygen of which has been replaced by sulphur, dispersing in an inert ordinarily liquid medium 55 such a compound of a metal different from those containing as metallic constituents only alkali metals and alkali earth metals as is capable of entering into reaction with said thio salt with the formation of a metal sulphide, and combining the dispersion of the said thio salt with the dispersion of said metal compound so that reaction therebetween takes place.

6. The process which comprises treating combustible carbonaceous materials heavier than gasoline under conditions to effect destructive hydrogenation and in the presence of a metal sulphide catalyst which has been prepared by dispersing a thio salt containing ammonium as cation in water, said thio salt being of the form 60 of a salt of an oxygen acid of a metallic element the oxygen of which has been replaced by sulphur, dispersing in water such a compound of a heavy metal substantially free from alkali metals and alkaline earth metals as is capable of entering into reaction with said thio salt with the formation of a metal sulphide, and combining the dispersion of the said thio salt with the dispersion of said metal compound so that reaction therebetween takes place.

7. The process which comprises treating combustible carbonaceous materials heavier than gasoline under conditions to effect destructive hydrogenation and in the presence of a metal sulphide catalyst which has been prepared by dispersing a thio salt containing ammonium as cation in an organic solvent, said thio salt being of the form of a salt of an oxygen acid of a metallic element the oxygen of which has been replaced by sulphur, dispersing in an organic solvent such a compound of a heavy metal substantially free from alkali metals and alkaline earth metals as is capable of entering into reaction with said thio salt with the formation of a metal sulphide, and combining the dispersion of the said thio salt with the dispersion of said metal compound so that reaction therebetween takes place.

MATHIAS PIER.  
WALTER SIMON.  
PAUL JACOB.